# EUROPEAN PATENT SPECIFICATION

(11) **EP 0 365 682 B1**
(45) Date of publication and mention of the grant of the patent: **02.08.1995**
(21) Application number: 89903523.2
(22) Date of filing: 17.03.1989
(51) Int. Cl.: C23C 2/06, C23C 2/20, C23C 2/28, C23C 22/78

(54) **HOT-DIP ZINC-ALUMINUM ALLOY COATED STEEL SHEET FOR PREPAINTED STEEL SHEET, PROCESS FOR PRODUCING THE SAME AND PREPAINTED STEEL SHEET**
MIT ZINK-ALUMINIUM-LEGIERUNG BESCHICHTETES FEUERVERZINKTES STAHLBLECH FÜR VORGESTRICHENES STAHLBLECH UND VERFAHREN ZU SEINER HERSTELLUNG
FEUILLE D'ACIER REVETUE D'UN ALLIAGE EN ZINC-ALUMINIUM PAR IMMERSION EN BAIN CHAUD POUR FEUILLE D'ACIER PREPEINTE, PROCEDE DE PRODUCTION DE LA FEUILLE REVETUE ET DE LA FEUILLE D'ACIER PEINTE D'AVANCE

(30) Priority: 12.04.1988 JP 89998/88
(43) Date of publication of application: 02.05.1990
(73) Proprietor: TAIYO STEEL CO., LTD., Chuo-ku Tokyo 103 (JP)
(72) Inventor: KAMEYA, Toru, Chiba 281 (JP); SHIMIZU, Hisanori, Chiba 281 (JP); TAKAGI, Masaaki, Aichi 456 (JP); OKUZAKI, Yuuji, Chiba 285 (JP); OHTA, Koji, Chiba 273 (JP)
(74) Representative: Sheard, Andrew Gregory
(86) International application number: JP8900291
(87) International publication number: WO8909844

(56) References cited:
- EP-A- 0 038 904
- DE-A- 1 936 633
- DE-A- 3 242 625
- US-A- 3 320 040
- US-A- 3 369 923
- Patent Abstracts of Japan, vol. 10, no. 63 (C-332)(2120), 13 March 1986; & JP-A-60200953 (KAWASAKI SEITETSU K.K.) 11 October 1985
- Patent Abstracts of Japan, vol. 9, no. 17 (C-262)(1740), 24 January 1985; & JP-A-59166663 (SUMITOMO DENKI KOGYO K.K.) 20 September 1984
- Patent Abstracts of Japan, vol. 8, no. 11 (C-205)(1448), 18 January 1984; & JP-A-58177446 (NITSUSHIN SEIKOU K.K.) 18 October 1983
- Patent Abstracts of Japan, vol. 9, no. 52 (C-269)(1775), 6 March 1985; & JP-A-59193258 (SUMITOMO KINZOKU KOGYO K.K.) 1 November 1984
- Patent Abstracts of Japan, vol. 9, no. 96 (C-278)(1819), 25 April 1985; & JP-A-59226161 (SHIN NIPPON SEITETSU K.K.) 19 December 1984
- Patent Abstracts of Japan, vol. 9, no. 233 (C-304)(1956), 19 September 1985; &
- JP-A-6092483 (KAWASAKI SEITETSU K.K.) 24 May 1985
- Patent Abstracts of Japan, vol. 9, no. 184 (C-294)(1907), 30 July 1985; & JP-A-6052569 (TAIYOU SEIKOU K.K.) 25 March 1985
- Patent Abstracts of Japan, vol. 12, no. 353 (C-530)(3200), 21 September 1988; &JP-A-63111163 (KAWASAKI STEEL CORP.) 16 May 1988

## Description

The present invention relates to prepainted steel sheets having excellent properties suitable for use as constructions materials such as roof materials and wall materials as well as household electric appliances, hot-dip zinc-aluminium alloy coated steel sheets having properties superior to those of conventional ones and suitable for use as the sheets of the prepainted sheets and a process for producing them.

JP-A-60/52569 discloses a hot-dip tin-plated steel sheet that is prepared using a plating bath containing from 0.03 to 3.5% aluminium, silicon in the ratio 1:30 to aluminium and/or at least 0.01 to 1.5% of magnesium, manganese and copper.

US-A-3369923 describes a process of galvanising a metal strip by applying a zinc coating. During application of galvanised coating a temperature of as low as 177°C (350°F) can be employed, and the strip should enter the bath at a temperature of no higher than 449°C (840°F). The bath contains from 0.05 to 0.10% aluminium.

EP-A-0038904 describes a process for producing a hot galvanised steel strip by coating a strip substrate with a molten zinc based alloy. On page 23 it is disclosed that a wiping gas may be employed, which has a set having a thickness of 0.6 mm and located at 10 mm from the surface of the melted zinc based alloy coating, under a pressure of 1.0 kg/cm². JP 58-177446 refers to plating steel plates with an alloy by hot dipping, where the hot dipping bath is at a temperature equal to or less than the steel plate.

Steel sheets coated with zinc (Zn) or prepainted steel sheets produced therefrom have been used in construction materials or household electrical appliances. Further steel sheets coated with zinc-aluminium (Zn-A1) alloy attract attention as materials taking the place of Zn coated steel sheets, since they have corrosion resistance, etc. superior to those of the Zn coated ones.

Various processes have been proposed heretofore for producing the Zn-Al alloy coated steel sheets. These processes include one comprising the use of a coating bath comprising 5 to 25 wt.% of Al, 0.1 wt.% or less of Pb and the balance of Zn (see Japanese Patent Publication No. 25220/1976); one comprising the use of a coating bath comprising more than 3.5 wt.% but not more than 10 wt.% of Al, and Mg, Be, Ti and Cu each in a specified range of a small amount relative to the concentration of Pb, Sn or both of them in the coating bath (see Japanese Patent Publication No. 47055/1978); one comprising the use of a coating bath comprising 3 to 15 wt.% of Al, about 85 to 97 wt.% of Zn and small amounts of rare earth elements (see Japanese Patent Publication No. 500475/1982); and one comprising the use of a coating bath comprising 0.05 to 2.0 wt.% of Al, 0.01 to 0.1 wt.% of Mn and the balance of Zn and unavoidable impurities (see Japanese Patent Publication No. 32700/1985).

A principal object of these processes is to reduce the weight loss of the coated steel sheets due to corrosion by the addition of Al.

The loss due to corrosion of the coated steel sheets in exposure tests in outdoor is usually reduced as the Al concentration in the coating bath is increased and, therefore, the corrosion resistance of the sheets is improved. However, an alloy layer formed on the interface with iron becomes thicker and the adhesion and the workability of the coating layer are seriously reduced as the Al concentration is increased.

Methods have been proposed to solve these problems by adding small amounts of various elements. However, they have problems that the use of the limited kinds of elements in limited amounts is troublesome, that the coating pot must be exchanged in order to switch over the coating bath and that the appearance of the coated steel sheet surface is impaired. Under these circumstances, the development of a process for producing coated steel sheets which can satisfy the required qualities with as little as possible elements added is demanded.

The following properties are required of Zn-Al alloy coated steel sheets, particularly those to be used as sheets for prepainted steel sheets from the viewpoint of the use of them:
(1) the corrosion resistance of the steel sheet surface is improved,
(2) a self-sacrificing rust-preventive power of Zn for that part of iron which is exposed when the steel sheet is cut is retained,
(3) no crack is formed in a bent part of the steel sheet in the working step,
(4) the coating layer has an excellent adhesion which is not reduced with time, and
(5) the surface smoothness is excellent.

The present applicant proposed a coated steel sheet for prepainted galvanized steel sheets which is produced by coating a steel sheet with hot dipping bath comprising 0.3 to 3.5 wt.% of Al and the balance of Zn and unavoidable impurities (see Japanese Patent Application No. 159469/1983).

It is apparent from the phase diagram of Zn-Al alloy that the eutectic point is realized when the alloy comprises 5 wt.% of Al (95 wt.% of Zn). When the Al content is deviated to some extent from 5 wt.%, the texture of the solidified alloy is quite different from that of the 5 wt.% Al alloy unless it is quenched at a very high speed. The Al-Zn alloy having 5 wt.% Al content is eutectic and, therefore, its melting point is low and Al and Zn are dispersed homogeneously irrespective of the cooling rate. However, when the Al content is less than 5 wt.%, for example, 1 wt.%, a primary crystal of Zn containing only very small amount of the Al component is formed in the coating layer and the majority of the Al component remains in the finally solidified grain boundary. Thus no coating layer having homogeneous composition is formed. It has been believed that an Al-Zn alloy having an Al content of 5 wt.% is advantageous for homogeneously dispersing Al and Zn and for giving a stable texture.

### Disclosure of Invention:

After investigations of an Al-Zn alloy having an Al content of 0.3 to 3.5 wt.% which is less than the above-described value, 5 wt.%, the inventors have completed the present invention. According to the present invention, the qualities and properties required of Zn-Al alloy coated steel sheets are satisfied or further improved.

Thus the invention relates to a process for the preparation of a hot-dip zinc-aluminium alloy coated steel sheet suitable for a prepainted steel sheet, comprising coating a steel sheet in a hot dipping bath comprising 0.3 to 3.5 wt.% of Al, 100ppm or less of Pb and the balance of Zn and unavoidable impurities, wherein the temperature of the steel sheet dipped in the hot dipping bath is lower than that of the hot dipping bath by 10 to 80°C, taking the steel sheet out of the hot dipping bath and reheating the coated steel sheet to a temperature above the melting temperature of the coating layer. Hot-dip zinc-aluminium alloy coated steel as prepared in claims 1-5 and/or a prepainted sheet as prepared in claim 6 is also the subject of the invention.

In the accompanying drawings:
Figs. 1(a) to (c) are microphotographs of the metal textures on the surfaces of the coating layers formed in Example 5 of the present invention and according to a Comparative Example. They are X-ray images of Al on the surface obtained with EPMA. Figs. 1(a), 1(b) and 1(c) are microphotographs of the metal textures of the coating layer surfaces obtained when (steel sheet temperature at dipping time) - (bath temperature) was 20°C, -20°C and -80°C, respectively.
Figs. 2(a) and (b) show the concentration distribution of Fe, Zn and Al in the thickness direction of the hot-dip zinc-aluminum alloy coated steel sheets produced in Example 5 of the present invention. They show the concentration distributions obtained when (steel sheet temperature at dipping time) - (bath temperature) was 20°C and -80°C, respectively.
Fig. 3 is a schematic drawing of the hot dipping equipment used in Example 6 of the present invention.
Figs. 5(a) and (b) show the thickness distributions of the coating layers, wherein Fig. 5(a) shows that of the coating layer having a surface not reheated (Comparative Example) and Fig. 5(b) shows that of the deposit coating layer having a surface reheated at 460°C (Example 7 of the present invention). (Figures 4 and 6 have been deleted).

### Best Mode for Carrying Out the Invention:

The present invention also relates to a prepainted steel sheet produced from the above-described Zn-Al alloy coated steel sheet.

The prepainted steel sheets are those previously painted with a paint. They are produced continuously on a large scale by painting galvanized steel sheets or zinc alloy coated steel sheets with a roll coater usually after chemical conversion treatment. The demand for them as starting materials for construction materials household electric appliances, business machines, etc. is now increasing, since they have excellent, uniform qualities, they can be supplied in large amounts and no painting is necessary after application.

The properties required of the prepainted steel sheets are mainly adhesion, corrosion resistance, workability, weather resistance and scratch resistance. However, it is quite difficult to satisfy all o the required properties with only one paint.

Thus it was a usual practice to classify paints into two groups in the prior art, i.e. those for under-painting which could impart adhesion and corrosion resistance and paints for toppainting which could impart workability, weather resistance and scratch resistance to further improve the qualities and properties of the prepainted steel sheets. These paints were applied by the so-called two-coat two-bake process wherein the sheets were baked after application of the under-painting paint and baked again after application of the toppainting paint in order to improve the qualities of the prepainted steel sheets.

However, recently, durability over a period of as long as, for example, 10 or 20 years is demanded of the construction materials such as roof and wall materials in various cases.

The term "durability" as used herein means weather resistance and corrosion resistance. Namely, an excellent durability means that the color tone and gloss are substantially unchanged and no rust is formed in 10 or 20 years.

The excellent weather resistance can be given by using a paint having excellent properties against chalking and fading.

However, it is difficult to inhibit the rust formation over a long period of time.

The formation of red rust is often observed in a portion of roof or wall material worked by roll forming machine only several years after the construction, though the timing of the rust formation varies depending on the environmental conditions.

Such rust formation occurs even when the material is exposed to the outdoor for only a short period of time, since cracks are formed in the worked part already prior to the use and in an extreme case, the steel texture is exposed through the cracks formed in the coating layer.

To solve this problem, it is necessary to cover the coating layer with a painting film having such an excellent elongation that it can withstand the deformation in the course of working and to use a steel sheet having a coating layer having such an excellent workability that it is not cracked in the course of working.

The former requirement was satisfied by producing prepainted steel sheets or metal sheets having excellent corrosion resistance after intensive investigations. The inventors made investigations for the purpose of satisfying the latter requirement.

After intensive investigations made for the purpose of satisfying the latter requirement, the inventors have succeeded in the production of Zn-Al alloy coated steel sheets having excellent properties. After further investigations of prepainted steel sheets, the inventors have found that two-coat steel sheets having a performance equivalent to that of three-coat steel sheets can be produced when the Zn-Al alloy coated steel sheets prepared by the present invention are used.

The Al concentration is limited because when it exceeds 3.5 wt.%, the self-sacrifying anti-corrosive effect of Zn on iron is reduced while when it is insufficient, the effect of improving the corrosion resistance at the surface of the coating layer is unsatisfactory. With at least 0.3 wt.% Al concentration, the workability is also improved and this effect is remarkable when the Al concentration is 0.5 wt.% or higher.

The Pb concentration is limited because when it exceeds 100 ppm, the adhesion is reduced with time due to intercrystalline corrosion and consequently the corrosion resistance which is particularly important for the prepainted steel sheet is damaged. With 100 ppm or less of Pb, stable adhesion which is not reduced with time can be obtained. With an Al concentration of 0.3 to 3.5 wt.% and a Pb concentration of 100 ppm or less, a zinc-aluminium alloy coated steel sheet which does not cause reduction in adhesion with time, has an excellent workability and is quite suitable for use as the sheet for a prepainted steel sheet can be obtained.

The temperature of the hot dipping bath may be one at which Zn and Al are molten to form a homogeneous melt, such as about 430 to 480°C.

The invention in a specific embodiment encompasses a hot-dip zinc-aluminum alloy coated steel sheet for a prepainted steel sheet, which is produced by coating in a hot dipping bath comprising 0.3 to 3.5 wt.% of Al, 1/100 to 1 part, per part of Al, of Si, 100 ppm or less of Pb and the balance of Zn and unavoidable impurities.

Although a hot-dip zinc-aluminium alloy coated steel sheet having excellent workability and adhesion after aging can be obtained when the Al concentration is in the range of 0.3 to 3.5 wt.% and the Pb concentration is 100 ppm or less, it is further preferred to add 1/100 to 1 part, per part of Al, of Si. The addition of Si serves to inhibit the formation of the alloy layer at the interface between the steel sheet and the coating layer to thereby make the formation of a thin alloy layer possible. Thus, a zinc-aluminium alloy coated steel sheet having further improved workability and adhesion after aging can be obtained.

The Si concentration is limited because when it is as low as about 1/200 of the Al concentration, no improvement in the workability or adhesion can be obtained. Another reason is that the control of the addition of Si in an amount of as small as 1/200 of Al is difficult, since the Al concentration is as low as 0.3 wt.% or less. The lower limit of the Si concentration is thus 1/100 of the Al concentration.

The Al concentration is limited for the same reasons.

The invention in a specific embodiment also encompasses a hot-tip zinc-aluminium alloy coated steel sheet or a prepainted steel sheet, which is produced by coating in the same hot dipping bath as that described above, which further contains 0.01 to 1.5 wt.% of one or more metals selected from the group consisting of Mg, Mn and Cu.

When metallic elements effective in improving the corrosion resistance of the galvanized steel sheet, such as Mg, Mn or Cu, are added to the bath, the effects of the resent invention, i.e. satisfactory workability, corrosion resistance and adhesion after aging are further improved. With 0.01 wt.% or more of the metallic elements, the effects can be obtained. The addition of the metallic elements in an amount larger than 1.5 wt.% is not preferred from the viewpoint of the cost or efficiency of working. Mg, Mn and Cu may be used alone or in combination of them. By adjusting the amount of Pb to 100 ppm or less, a stable adhesion after aging can be attained.

The invention relates, in a specific embodiment, to a process for producing a hot-dip zinc-aluminium alloy coated steel sheet for a prepainted steel sheet, wherein the temperature of the starting steel sheet dipped in the hot dipping bath is lower than that of the bath in the step of coating in the hot dipping bath. One feature of the invention resides in that the temperature of the steel sheet dipped in the hot dipping bath at the dipping time is adjusted to a temperature lower than that of the bath. The temperature of the steel sheet to be dipped in the hot-dip Zn-Al alloy coating bath is adjusted to a temperature lower than the bath temperature by 10 to 80°C. By this process, a hot-dip zinc-aluminium alloy coated steel sheet having an excellent surface corrosion resistance and a high power of protecting the edge of the steel from rust is obtained. Also the corrosion resistance in a bent part is improved.

Usually in the production of a hot-dip coated steel sheet in hot dipping equipment provided with a continuous annealing furnace, the temperature of the steel sheet to be dipped in a hot dipping bath is kept higher than a temperature of the bath from the viewpoints of the adhesion and the heating effect of the bath. Since the steel sheet is thicker than the coating layer and the temperature of the steel sheet is high, the cooling of the coating layer starts with its surface and the interface of the coating layer with the steel sheet is solidified layer. Consequently, the Al concentration is high in the interface and the thickness of the alloy layer is increased to thereby reduce the workability and the self-sacrificing anti-corrosive effect on the steel, while the Al concentration on the coating layer surface is low to reduce the corrosion resistance.

The temperature of the steel sheet dipped in the hot dipping bath is kept 10-80°C below the bath temperature contrary to the conventional processes in order to initiate the cooling of the coating metal on the side facing to the steel sheet. By this process, the inventors have succeeded in reducing the Al concentration on the interface side and reducing the amount of the alloy layer formed. In this process, the self-sacrificing anticorrosive power (resistance to the initial red rust formation) of Zn is retained. Further, since the alloy layer formed is thin, no crack is formed in the bent part.

On the other hand, the Al concentration in the surface region of the coating layer is increased and, therefore, the corrosion resistance of the surface is improved (namely, the weight loss due to corrosion is reduced).

In the present invention the temperature of the steel sheet to be dipped in the hot-dip Zn-Al alloy coating bath is kept at 10-80°C below the temperature of the bath and the temperature of the steel sheet to be pulled out of the bath is kept below the bath temperature as far as possible in order that the solidification of the coating layer be started with the part in contact with the steel sheet and is completed as soon as possible. Such a process has never been applied to a bath of 0.3-3.5 wt.% Al and 100 ppm of Pb, the balance being Zn.

The hot dipping bath temperature is such that Zn and Al are molten to form a homogeneous melt, for example, about 430 to 480°C.

The temperature of the steel sheet to be dipped in the hot dipping bath is kept below the bath temperature by 10 to 80°C. For example, when the bath temperature is 480°C, the temperature of the steel sheet to be dipped in the hot dipping bath is kept in the range of 400 to 470°C. This is because when the temperature of the steel sheet to be dipped in the hot dipping bath is equal to or lower than the bath temperature and also that of the steel sheet to be pulled out of the bath is lower than the bath temperature, the steel sheet will have a thickness larger than that of the coating layer and, since the temperature of the sheet pulled out is lower than the bath temperature, the cooling of the coating layer is started with the inner face and the Al concentration is high in the surface layer, since Al tends to concentrate in a part which is solidified later. However, when the temperature of the steel sheet is lower by more than 80°C, the adhesion of the coating layer is reduced and the lowering in the bath temperature is serious to thereby increase the operation cost.

The Al concentration in the grain boundaries where solidification occurs later is higher than that in the grain centers where crystallization occurs in an initial stage. In practice, the Al concentration in the surface layer is uneven and it forms a honey-comb pattern in which parts of a relatively low Al concentration are surrounded by parts of a high Al concentration. However, the area of the parts of the high Al concentration is large enough for improving the corrosion resistance of the whole surface.

Although the Al-Zn crystals are formed also in the surface layer upon cooling of the surface layer, also the homogeneous dispersion of Al in the surface layer is accelerated, since the cooling velocity of the whole coating layer is increased by dipping the steel sheet kept at a low temperature. Further the bath is preferably a low temperature bath.

As described above, the Pb concentration in the hot dipping bath must be controlled to 100 ppm or less in order to obtain an excellent adhesion after aging. However, when the Pb concentration is 500 ppm or less, the surface of the coating layer has a ripping pattern to impair the appearance thereof unfavorably. After intensive investigations made for the purpose of eliminating such a pattern from the surface, the inventors have succeeded in obtaining an excellent appearance by controlling the amount of the molten zinc-aluminum alloy deposit with a gas wiping type of equipment under conditions comprising a nozzle slit clearance of 0.6 to 2.4 mm, a distance between front and back nozzles of 10 to 40 mm and an ejecting pressure of gas of 0.1 to 2.0 kg/cm².
These values are limited for the following reasons:

### 1. Nozzle slit clearance:

When the lower limit is less than 0.6 mm, the secondary pressure variation of the gas is too much to obtain a consistent appearance.

When the upper limit exceeds 2.4 mm, the amount of the gas is too much and the energy loss is serious.

### 2. Distance between front and back nozzles:

The lower limit is 10 mm, because when it is less than 10 mm, the vibrating strip is apt to be brought into contact with the nozzle to cause troubles.

The upper limit is 40 mm, because a shorter distance gives a better result and the appearance is impaired when it exceeds 40 mm.

### 3. Ejecting pressure of gas:

The lower limit is 0.1 kg/cm² because when it is below 0.1 kg/cm², the amount of the deposition cannot be controlled.

The upper limit is 2.0 kg/cm² because when it exceeds 2.0 kg/cm², the energy loss is large and a more consistent appearance can be obtained with a lower pressure.

The control of the amount of the deposition is necessary in order to conform to Z 27 specified in JIS G 3302 or G 90 specified in ASTM A 525.

In the invention the hot-dip zinc-aluminium alloy coated steel sheet is reheated to a temperature above the melting temperature or the coating layer.

The reheating temperature is preferably 420°C or higher, because the appearance of the sheet can be improved at such a high temperature.

Although the reheating temperature is preferably 420°C or above, a high temperature is not preferred from the viewpoints of both energy and equipment cost. Thus, a temperature in the range of 420°C to 560°C is more preferred.

Since the temperature of the steel sheet is lower than that of the coating layer in the step of melting the coating layer surface again and, therefore, the recrystallization of the molten coating metal starts with the side in contact with the steel sheet. The alloy layer formed between the steel sheet and the coating layer is not molten again, because it has a high melting point and therefore, the Al distribution in the alloy layer is kept unchanged and the adhesion of the coating layer is kept high.

Preferably the hot-dip zinc-aluminium alloy coated steel sheet is cooled to the solidifying point thereof at a rate of at least 10°C/sec.

The lower limit of the cooling rate is 10°C/sec, because stable corrosion resistance can be obtained at a cooling rate of at least 10°C/sec. Although the higher limit thereof is not limited, a cooling race of 150°C/sec or less is desirable from the viewpoints of the energy cost and equipment.

The invention in a specific embodiment relates to a prepainted steel sheet having excellent workability and corrosion resistance which comprises the hot-dip zinc-aluminum alloy coated according to the process of the present invention, a layer formed thereon by chemical conversion treatment and further a surface painting film layer formed thereon.

The surface painting film layer comprises those of one-coat, two coat, three-coat, four-coat type, etc. Usually, a two-coat layer is used.

The present invention will be described in detail with reference to a two-cost surface painting film layer.

First, an under-painting paint is applied to the sheet and baked.

The sheet used is the hot-dip zinc-aluminum alloy coated steel sheet. The sheet may have a layer formed by chemical conversion treatment having a thickness of about 0.1 to 5 ».

The chemical conversion treatment is conducted in order to improve the corrosion resistance of the sheet and the adhesion of the paint to the steel sheet. The chemical conversion treatments include, for example, a treatment with a phosphate such as zinc phosphate, iron phosphate, manganese phosphate or cobalt phosphate, and a treatment with a chromate such as electrolytic chromate treatment and applied chromate treatment.

As the under-painting paints, those ordinarily used for the production of prepainted steel sheets can be used. They include, for example, paints prepared by mixing coloring pigment, rustproof pigment, body, etc. in a resin solution mainly comprising a resin such as epoxy, oil-free polyester, acrylic or urethane resin. Among them, an under-painting paint mainly comprising the epoxy resin which has excellent adhesion and corrosion resistance or the oil-free polyester resin which has also a good workability is preferred. The thickness of the under-paint is 1 to 15 », preferably 2 to 12 », because the corrosion resistance and scratch resistance are further improved with a thickness of at least 2 » and the workability is further improved with that of 12 » or less. When the thickness exceeds 12 », the cost is increased.

The rustproof pigment may contain 5 to 35% of at least one of strontium chromate, zinc chromate, red lead, zinc plumbate, calcium plumbate, lead cyanamide, basic lead chromate, basic lead silicochromate, basic zinc molybdate and calcium zinc molybdate depending on the use and environments. With at least 5% of this pigment, the rust formation in an early stage can be completely inhibited and no blister is formed with 35% or less thereof.

After formation of the under-paint, a top-paint paint is applied thereto and baked to form a topcoat. The top-painting paint comprises preferably acrylic resin, oil-free polyester resin, silicone polyester resin, silicone acrylic resin, alkyd resin, polyurethane resin, polyimide resin, polyamide resin, fluororesin or the like. The thickness of the top-paint is 8 to 50 », preferably 10 to 45 », because the scratch resistance, workability and weather resistance are improved with the thickness of at least 10 » but the cost is increased when the thickness is beyond 45 ».

When the Pb concentration exceeds 100 ppm, the adhesion after aging is reduced due to intercrystalline corrosion and, as a result, the corrosion resistance of a worked part which is important particularly in the prepainted steel sheet is also reduced. The concentrations of Al and Pb must be thus limited in order to produce the prepainted steel sheet having excellent properties.

In a preferred embodiment a prepainted steel sheet has a chemical conversion layer formed by treating the sheet with a chromic acid solution containing silica having an average particle diameter of 50 »m and specific surface area of 200 m²/g in such a manner that the amount of the coating film after drying will be 50 to 250 mg/m² to impart an excellent scratch resistance.

Chromic acid solution containing silica having an average particle diameter of 50 »m may be used. The smaller the average particle diameter of silica, the better the workability and adhesion, though the scratch resistance is not improved when the average particle diameter is too small. When the average particle diameter is too large, the particles are liable to be precipitated disadvantageously.

The specific surface area of silica in the chromic acid solution may be 200 m²/g. Although it varies depending on the average particle diameter, no scratch resistance can be obtained when the specific surface area is excessively small.

The chemically converted layer is formed with the above-described chromic acid solution in such a manner that the amount of the coating film after drying will be 50 to 250 mg/m². With at least 50 mg/m² of the film after drying, both the scratch and corrosion resistances are improved and with 250 mg/m² or less thereof, the workability, adhesion and scratch resistance are improved.

### (Examples)

The following Examples will further illustrate the present invention.

The materials to be coated were low-carbon aluminum killed steel sheets (0.8 mm x 914 mm x coil) in all the cases. The sheets were hot-dip coated with Zn-Al alloy with Sendzimir continuous zinc coating equipment.

The invention stated in Claim 1 of the present application will be described with reference to Examples.

### Example 1

Hot-dip zinc-aluminum alloy coated steel sheets were produced with hot dipping baths having various Al concentrations and the workability thereof was examined in order to confirm the effects obtained by the addition of Al according to the present invention.

The conditions were as follows:

| | |
|---|---|
| sheet thickness: | 0.8 mm |
| bath temperature: | 460°C |
| dipping time in the bath: | 4 sec |
| amount of deposition: | 120 to 260 g/m² |
| Pb concentration: | 50 ppm |

### (1) Test method:

The 0T and 2T bending test methods according to JIS G 3312 were employed. The term "0T bend" and "2T bend" refer to the bends realized when a steel sheet having a thickness of the base metal of T is bend with a hand vise or other suitable means to give an inner diameter of the bend of 0T and 2T, respectively. The cracks of the coating layer in the bend part were examined and the results were classified into five groups. The standard is shown in Table 1 and the results are shown in Table 2.

**Table 1**

| (Standard of evaluating degree of cracking) | |
|---|---|
| | Standard |
| 5 | No crack formed. |
| 4 | Extremely slight crack formation observed. |
| 3 | Slight crack formation observed. |
| 2 | Crack formation distinct. |
| 1 | Crack formation remarkable. |

**Table 2**

| | Aℓ wt% | Workability | |
|---|---|---|---|
| | | 0T | 2T |
| Comparative | 0 | 1 | 1 |
| | 0.1 | 1 | 2 |
| | 0.2 | 2 | 3 |
| Present invention | 0.3 | 3 | 4 |
| | 0.5 | 4 | 5 |
| | 1.0 | 4.5 | 5 |
| | 1.5 | 4.5 | 5 |
| | 2.0 | 4.5 | 5 |
| | 2.5 | 5 | 5 |
| | 3.0 | 5 | 5 |
| | 3.5 | 5 | 5 |
| Comparative | 4.0 | 5 | 5 |
| | 5.0 | 5 | 5 |
| | 10.0 | 3 | 4 |
| | 15.0 | 2 | 3 |
| The numerals in Table 2 are the averages of the results. | | | |

### Example 2

Hot-dip zinc-aluminum alloy coated steel sheets were produced with hot dipping baths having various Pb concentrations and the prolonged adhesion thereof was examined in order to confirm the effects of Pb added according to the present invention.

The conditions were as follows:

| | |
|---|---|
| sheet thickness: | 0.8 mm |
| bath temperature: | 460°C |
| dipping time in the bath: | 4 sec |
| amount of deposition: | 120 to 260 g/m² |

### (2) Test method (adhesion after aging or adhesion after working:

A paint was applied to the test pieces in a thickness of about 5 » and then baked in order to prevent formation of white rust. The test pieces were immersed in hot water kept at 80°C for 3 days and taken out. The painting film was removed with a stripping agent. A semi-spherical steel mass weighing 5 kg and having a radius of 3/4 inch was dropped from a height of 500 mm. An adhesive tape was applied to the projecting coated surface to forcedly strip it to thus determine the adhesion of the coating layer. The standard is shown in Table 3 and the results are shown in Table 4.

**Table 3**

| (Standard of adhesion after aging or adhesion after working) | |
|---|---|
| | Standard |
| 5 | No peeling observed. |
| 4 | Extremely slight peeling observed. |
| 3 | Slight peeling observed. |
| 2 | Peeling distinct. |
| 1 | Peeling remarkable. |

The following Example 3 illustrates a preferred embodiment of the invention.

### Example 3

Hot-dip zinc-aluminum alloy coated steel sheets were produced with hot dipping baths containing various amounts of Si and the workability and adhesion thereof were examined in order to confirm the effects obtained by the addition of Si.

### (Test method)

A semi-spherical steel mass weighing 5 kg and having a radius of 3/4 inch was dropped from a height of 500 mm and an adhesive tape was applied to the projecting coated surface to forcedly strip it to thus determine the adhesion of the coating layer. The results are shown in Table 5. The standard is the same as that shown in Table 3.

The conditions were as follows:

| | |
|---|---|
| sheet thickness: | 0.8 mm |
| bath temperature: | 460°C |
| dipping time in the bath: | 4 sec |
| amount of deposition: | 120 to 260 g/m² |
| Pb concentration: | 50 ppm |

In Table 5, the results of 0T crack formation according to the bending test are shown in the upper row and those of 0T tape tests on adhesion after working are shown in the lower row.

When the Al concentration is in the range of 0.3 to 3.5 wt.% and the Pb concentration is not higher than 100 ppm, hot-dip zinc-aluminum alloy coated steel sheets having excellent workability and adhesion after aging can be obtained. It is preferred, however, to add 1/100 to 1 part of Si per part of Al to control the formation of the alloy layer and, therefore, to form only a thin alloy layer. By this process, a hot-dip zinc-aluminum coated steel sheet further improved in adhesion after aging can be obtained. When only 1/200 part of Si is added per part of Al, no improvement is observed.

It was thus confirmed that when the Al concentration was 0.3 to 3.5 wt.%, Pb concentration was 100 ppm or less and Si concentration was 1/100 to 1 part per part of Al, an intended hot-dip zinc-aluminum alloy coated steel sheet which has excellent workability and adhesion can be obtained.

The following Example 4 illustrates a preferred embodiment of the invention.

### Example 4

Hot-dip zinc-aluminum alloy coated steel sheets were produced with hot dipping baths containing various amounts of Mg, Mn or Cu and the corrosion resistance and adhesion after aging thereof were examined in order to confirm the effects obtained by the addition of it.

The conditions were as follows:

| | |
|---|---|
| sheet thickness: | 0.8 mm |
| bath temperature: | 460°C |
| dipping time in the bath: | 4 sec |
| amount of deposition: | 120 to 260 g/m² |
| Pb concentration: | 50 ppm |

### (Test method)

Test pieces prepared under the conditions shown in Table 7 were subjected to the chromate treatment. An epoxy resin under-paint having a thickness of 5 » and then a silicone polyester resin top-paint having a thickness of 15 » were formed. After baking, they were subjected to a salt spray best according to JIS Z 2371 and the corrosion resistance in the 0T part of each of the prepainted steel sheets was examined. The results are shown in Table 7. The standard is shown in Table 6.

**Table 6**

| (Standard of evaluation of corrosion resistance) | |
|---|---|
| | Standard |
| 5 | No white rust formed. |
| 4 | Extremely slight white rust formation observed. |
| 3 | Slight white rust formation observed. |
| 2 | White rust formation distinct. |
| 1 | White rust formation remarkable. |

The adhesion after aging was tested in the same manner as that of Example 2 and the results were evaluated according to the standard shown in Table 3.

When a metallic element such as Mg, Mn or Cu capable of improving the corrosion resistance of the galvanized steel sheet was added to the hot dipping bath, the effect of the present invention could be further improved. The effective concentration of the metallic element was 0.01 wt.% or higher. A combination of Si with Mg, Mn or Cu is also usable. By controlling the Pb concentration below 100 ppm, a stable adhesion after aging could be obtained.

The following Example 5 will illustrate the invention stated in Claim 1 of the present application.

### Example 5

Hot-dip zinc-aluminum alloy coated steel sheets were produced at various steel sheet temperatures and hot dipping bath temperatures as shown in Table 10 and the workability and corrosion resistance thereof were examined in order to confirm the effects of the present invention.

The results are shown in Table 10.

In this example, the temperature difference between the steel sheet and the bath was controlled to be 0 to 80°C to reduce the energy required to maintain the bath temperature.

### (Test methods)

### Surface corrosion resistance test

The four edges of each of the test pieces having a size of 60 mm x 60 mm were sealed by coating. Further the whole surface of the test piece other than the surface to be tested was also sealed by painting and then dried. The painting was conducted in such a manner that the area of the exposed surface of the test piece would be 50 mm x 50 mm. Then the test piece was thrown into a salt spray testing instrument and tested according to JIS Z 2371. After the completion of the test conducted for 100 Hr., the test piece was taken out, corrosion products were removed from the exposed surface thereof and the test piece was weighed. The loss due to corrosion (g/m²) was determined by dividing the difference in weight between that before the test and that after the test with the area of the test surface. The standard is shown in Table 8.

**Table 8**

| (Standard of evaluation of surface corrosion resistance) | |
|---|---|
| | Standard |
| 5 | Loss due to corrosion 50 g/m² or less |
| 4 | Loss due to corrosion 50 ∼ 75 g/m² |
| 3 | Loss due to corrosion 76 ∼ 100 g/m² |
| 2 | Loss due to corrosion 101 ∼ 125 g/m² |
| 1 | Loss due to corrosion 126 g/m² or above |

### Initial red rust test on edge

The test piece was placed in a salt spray testing instrument for 160 Hr. and red rust formed on the edges thereof was examined. The salt spray test was conducted according to JIS Z 2371. The standard of the examination of the red rust is shown in Table 9.

**Table 9**

| (Standard of examination of initial red rust formed on edge) | |
|---|---|
| | Standard |
| 5 | No red rust formed. |
| 4 | Extremely slight red rust formation observed. |
| 3 | Slight red rust formation observed. |
| 2 | Red rust formation distinct. |
| 1 | Red rust formation remarkable. |

The lower is the temperature of the steel sheet at the time of dipping into the bath, as compared with the bath temperature, the better is the corrosion resistance. The temperature difference between the sheet and the bath is less than 80°C to reduce the energy required to maintain the bath temperature.

The Al distribution on the coating layer surface at various steel sheet temperatus at dipping time is shown in Figs. 1. The samples used for the determination of this distribution were prepared under the following conditions:

| | |
|---|---|
| bath composition: | 1 wt.% of Al, 0.005 wt.% of Pb, 0.02 wt.% of Si and the balance of Zn |
| sheet thickness: | 0.8 mm |
| bath temperature: | 460°C |
| dipping time in the bath: | 4 sec |

Figs. 1(a), 1(b) and 1(c) are microphotographs of the metal textures obtained when (steel plate temperature at dipping time) - (bath temperature) was 20°C, -20°C and -80°C, respectively.

The Al distribution was determined with EPMA (EMX-SM 7; a product of Shimadzu Seisakusho Ltd.).

Fig. 2(b) shows the distributions of Fe, Zn and Al in the cross section of the hot-dip Zn-Al alloy coated steel sheet. This figure substantiates the fact that Al in the coating layer was distributed on the surface layer thereof to improve the corrosion resistance. Fig. 2(a) shows a cross section of the coating layer of a hot-dip Zn-Al alloy coated steel sheet produced by a conventional process. It is apparent that Al is distributed densely in the alloy layer.

It is thus apparent from the above figures that Al is distributed mostly in the surface layer of the coating layer in the products of the present invention unlike the products produced by a conventional process.

As described above, the present invention provides a hot-dip Zn-Al alloy coated steel sheet which has an excellent corrosion resistance of the coating layer, which is prevented from the initial red rust formation on the edges of the sheet and which has an excellent workability of the coating layer.

The following Example illustrates a preferred embodiment of the invention.

### Example 6

The steel sheet was pulled out of the hot dipping bath and the surface smoothness of the sheet was improved by means of a gas wiping type of equipment for controlling the amount of zinc deposit under conditions comprising a slit clearance of 0.6 to 2.4 mm, a distance between front and back nozzles of 10 to 40 mm and an ejecting of 0.1 to 2.0 kg/cm². The appearance (smoothness of the coating layer surface) of the produced hot-dip zinc-aluminum alloy coated steel sheet was examined.

The conditions were as follows:

| | |
|---|---|
| line speed: | 100 m/min |
| sheet thickness: | 0.8 mm |
| bath composition: | 1 wt.% of Al, 0.005 wt.% of Pb, 0.02 wt.% of Si and the balance of Zn |
| bath temperature: | 460°C |
| dipping time in the bath: | 4 sec |

Fig. 3 is a schematic drawing of the hot dipping equipment having a gas wiping type of means for controlling the amount of zinc deposit used in this Example.

### (Test method)

The appearance (smoothness) of the coating layer surface was evaluated on the basis of the standard shown in Table 11. The results are shown in Tables 12(1) and 12(2).

**Table 11**

| (Standard of evaluation of appearance smoothness of coating layer surface) | |
|---|---|
| | Standard |
| 5 | No ripple observed. |
| 4 | Extremely slight ripples observed. |
| 3 | Slight ripples observed. |
| 2 | Ripples distinct. |
| 1 | Ripples remarkable. |

Although the Pb concentration in the bath must be controlled to be 100 ppm or less to obtain an excellent adhesion after aging as described above, a Pb concentration of 500 ppm or less is not preferred for obtaining a good appearance, because a rough ripply pattern is formed on the surface with a Pb concentration of 500 ppm or less.

It is apparent from Tables 12(1) and 12(2) that a good appearance (smoothness) can be obtained by the invention stated in Claim 5 of the present application.

The control of the amount of the deposition is necessary in order to conform to Z 27 of JIS G 3302 or G90 of ASTM A525. The control thereof in the range of 50 to 400 g/m² is easy in Example 6.

### Example 7

The hot-dip zinc-aluminum alloy coated steel sheet was reheated to various temperatures shown in Table 14 which were above the melting temperature of the coating layer in order to make its surface smooth. The appearance (smoothness), thickness of the coating layer and Al distribution in the obtained hot-dip zinc-aluminum alloy coated steel sheet suitable for use as a material for a prepainted steel sheet were examined.

The conditions were as follows:

| | |
|---|---|
| sheet thickness: | 0.8 mm |
| bath temperature: | 460°C |
| dipping time in the bath: | 4 sec |
| amount of deposition: | 250 g/m² |
| bath composition: | 0.5 wt.% of Al, 0.005 wt.% of Pb, 0.01 wt.% of Si and the balance of Zn |

The standard of the evaluation of the appearance (smoothness) of the coating layer surface is shown in Table 11 and the results thereof are shown in Table 14.

**Table 14**

| | Reheating temp. (°C) | Smoothness of coating layer surface |
|---|---|---|
| Comparative | not reheated | 3 |
| | 380 | 3 |
| | 400 | 3 |
| Present invention | 420 | 4 |
| | 460 | 4.5 |
| | 500 | 4.5 |
| | 560 | 4.5 |
| The numerals of the evaluation results are the averages of the results. | | |

The surface smoothness was remarkably improved at a reheating temperature of 420°C or above.

The results of the determination of the thicknesses of the coating layers obtained without any reheating and with the reheating at 460°C are shown in Figs. 5.

It is apparent from Figs. 5 that the scattering in the thickness or the coating layer was narrow when the reheating was conducted according to the present invention. The scattering of the thickness of the coating layer was closely related to the appearance. Namely, the narrower the scattering, the less the formation of the ripples.

The thickness of the coating layer was determined with a micro-fluorescence X-ray device (SPT-157 SLS; a product of Seiko Denshi Co., Ltd.) with a beam diameter of 0.1 mm.

The distribution of Al atoms, etc. was examined with ESCA. The distribution of Fe, Zn and Al in the cross section of the coating layer on the hot-dip An-Al alloy coated steel sheet is shown in Table 15. The results support the fact that Al is distributed in the surface layer of the coating layer and the coated steel sheet of the present invention has an excellent corrosion resistance.

The conditions were as follows:

| | |
|---|---|
| sheet thickness: | 0.8 mm |
| bath temperature: | 460°C |
| dipping time in the bath: | 4 sec |
| amount of deposition: | 250 g/m² |
| bath composition: | 1 wt.% of Al, 0.003 wt.% of Pb, 0.01 wt.% of Si and the balance of Zn |

The ESCA instrument used was JPS-90 SX of JEOL, Ltd. The acceleration voltage (V) was 500 and the etching rate was 250 Å/min (in terms of SiO₂) (the etching rate of Zn is about 4 times as high as that of SiO₂).

**Table 15**

| (Atomic distribution change with depth from surface layer) | | | | | |
|---|---|---|---|---|---|
| | Depth | (Atomic %) Zn | (Atomic %) O | (Atomic %) C | (Atomic %) Aℓ |
| Surface layer | 0 | 3.21 | 40.58 | 38.95 | 17.25 |
| | 33Å | 5.62 | 57.94 | 8.17 | 28.25 |
| | 200 Å | 13.62 | 53.27 | 7.76 | 25.33 |
| | 1200 Å | 95.11 | 1.97 | 0.86 | 2.04 |
| | 6200 Å | 98.18 | 1.13 | 0.30 | 0.37 |
| | 11200 Å | 97.85 | 0.70 | 0.99 | 0.44 |

### Example 8

Hot-dip zinc-aluminum alloy coated steel sheets were produced with baths containing various amounts of Al and Pb in order to confirm the effects of Al and Pb added to the bath according to the present invention (Example 1). Each of them was used as the material sheet. It was treated with a chromate. An epoxy resin paint containing 15% of a rustproof pigment was applied thereto. After baking at 210°C for 35 sec, an under-paint having a dry thickness of 3 » was given. Then an oil-free polyester resin paint as the top-painting paint was applied thereto and baked at 220°C for 45 sec to form a top-paint having a dry thickness of 11 ».

The properties of the prepainted steel sheets thus prepared were examined. The results are shown in Table 17.

The workability was determined by the same 2T bending test method as that of Example 1 and the results were evaluated on the basis of the standard shown in Table 1.

The adhesion was determined also in the same manner as that of Example 1. Namely, after the 2T bending test, an adhesive tape was applied to the 2T part of the prepainted steel sheet and the forced stripping test was conducted. The results were evaluated on the basis of the standard shown in Table 3.

The corrosion resistance test was conducted according to JIS Z 2371 in the same manner as that of Example 4. The flat part and 2T part were subjected to the salt spray test (SST, 1000 Hr.). The results were evaluated on the basis of the standard shown in Table 6.

The workability adhesion and corrosion resistance were determined immediately after the preparation of the prepainted steel sheets and after six months.

When the Al concentration was in the range of 0.3 to 3.5 wt.%, the prepainted steel sheets having excellent properties could be obtained.

When the Pb concentration exceeded 100 ppm, the workability, adhesion and corrosion resistance were reduced with the elapse of time.

### Example 10 (Preferred Embodiment of the invention)

Hot-dip zinc-aluminum alloy coated steel sheets were prepared with hot dipping baths containing various amounts of Si in order to confirm the effect of Si added to the bath according to the present invention (Example 3). Each of them was used as the material sheet. It was treated with a chromate in the same manner as that of Example 9. An under-paint and then a top-paint were formed thereon to prepare a prepainted steel sheet in the same manner as that of Example 9. The workability, adhesion and corrosion resistance of the prepainted steel sheet were determined in the same manner as that of Example 9. The conditions and the results are shown in Table 18. Those baths having an Al and Si content outside claim 2 are marked as "comparative".

### Example 11 (Preferred Embodiment of the invention)

Hot-dip zinc-aluminum alloy coated steel sheets were prepared with hot dipping baths containing various amounts of Mg, Mn or Cu in order to confirm the effect of them added to the bath according to a preferred embodiment of the present invention (Example 4). Each of them was used as the material sheet. It was treated with a chromate. An epoxy resin paint containing 15% of a rustproof pigment was applied thereto. After baking at 210°C for 35 sec, an under-paint having a dry thickness of 3 » was given. Then an oil-free polyester resin paint as the top-painting paint was applied thereto and taked at 220°C for 45 sec to form a top-paint having a dry thickness of 11 ».

The workability, adhesion and corrosion resistance of the prepainted steel sheets were determined. The conditions and the results are shown in Table 19.

The workability was determined by the 2T bending test in the same manner as that of Example 1 and the results were evaluated on the basis of the standard shown in Table 1.

The adhesion in the 2T part of the prepainted steel sheet was determined also in the same manner as that of Example 9 and the results were evaluated on the basis of the standard shown in Table 3.

The corrosion resistance test was conducted according to JIS Z 2371 in the same manner as that of Example 4. The flat part and 2T part were subjected to the salt spray test (SST, 1000 Hr.). The results were evaluated on the basis of the standard shown in Table 6.

It is apparent from Table 19 that when 0.01 to 1.5 wt.% of one or more of Mg, Mn and Cu was(were) added to the bath, the workability, adhesion and corrosion resistance of the prepainted steel sheet were further improved. Those baths not falling within claim 3 are marked as "comparative".

### Example 12

Hot-dip zinc-aluminum alloy coated steel sheets were prepared by varying the bath temperature and the temperature of the steel sheet in order to confirm the effect of the temperature of the steel sheets to be dipped in the hot dipping bath according to the present invention (Example 5). Each of the sheets was used as the material sheet. It was treated with a chromate. An epoxy resin paint containing 15% of a rustproof paint was applied thereto. After baking at 210°C for 35 sec, an under-paint having a dry thickness of 3 » was given. Then an oil-free polyester resin paint as the top-painting paint was applied thereto and soaked at 220°C for 45 sec to form a top-paint having a dry thickness of 11 ».

The workability, adhesion and corrosion resistance of the prepainted steel sheets were determined. The conditions and the results are shown in Table 21.

The workability was determined by the 2T bending test in the same manner as that of Example 1 and the results were evaluated on the basis of the standard shown in Table 1.

The adhesion in the 2T part of the prepainted steel sheet was determined also in the same manner as that of Example 9 and the results were evaluated on the basis of the standard shown in Table 3.

The corrosion resistance test was conducted according to JIS Z 2371 in the same manner as that of Example 4. The flat part and 2T part were subjected to the salt spray test (SST, 1000 Hr.). The results were evaluated on the basis of the standard shown in Table 6.

It is apparent from Table 21 that when the temperature of the steel sheet to be dipped in the hot dipping bath is lower than the temperature of the bath, well-balanced, quite excellent workability, adhesion and corrosion resistance were obtained.

### Example 13

Hot-dip zinc-aluminum alloy coated steel sheets were prepared by the process stated in Claim 1 in which the reheating temperature was varied. The sheets were treated with a chromate and then painted and baked by the two-coat/two-bake process in the same manner as that of Example 9 to form prepainted steel sheets. The surface smoothness of the prepainted steel sheets was determined on the basis of the standard shown in Table 11 in the same manner as that of Example 6.

The smoothness test results and the reheating temperatures are shown in Table 23.

The bath composition was as follows:

| | |
|---|---|
| Al concentration | 0.5 wt.% |
| Pb concentration | 0.005 wt.% |
| Si concentration | 0.01 wt.% |
| Zn concentration | the balance |

The prepainted steel sheets having excellent smoothness could be thus prepared by the present invention.

**Table 23**

| | Reheating temp. (°C) | Smoothness after painting |
|---|---|---|
| Comparative | not reheated | 3 |
| Present invention | 380 | 3 |
| | 400 | 3 |
| | 420 | 4 |
| | 460 | 4.5 |
| | 500 | 4.5 |
| | 560 | 4.5 |
| The numerals of the smoothness test results are the averages of the results. | | |

### Example 14

The hot-dip zinc-aluminum alloy coated steel sheets prepared at various cooling speeds by the process stated in Claim 5 were used. Each of the sheets was treated with a chromate and then painted and baked by the two-coat/two-bake process in the same manner as that of Example 9 to form prepainted steel sheets. The workability, adhesion and corrosion resistance of the prepainted steel sheets were determined. The results are shown in Table 24 together with the cooling speeds.

The workability was determined by the 2T bending test in the same manner as that of Example 1 and the results were evaluated on the basis of the standard shown in Table 1.

The adhesion in the 2T part of the prepainted steel sheet was determined also in the same manner as that of Example 11 and the results were evaluated on the basis of the standard shown in Table 3.

The corrosion resistance test was conducted according to JIS Z 2371 in the same manner as that of Example 4. The flat part and 2T part were subjected to the salt spray test (SST, 1000 h). The results were evaluated on the basis of the standard shown in Table 6.

The bath composition was as follows:

| | |
|---|---|
| Al concentration | 1.0 wt.% |
| Pb concentration | 0.005 wt.% |
| Si concentration | 0.01 wt.% |
| Zn concentration | the balance |

The prepainted steel plates having excellent workability, adhesion and corrosion resistance could be prepared by the present invention.

**Table 24**

| | Cooling speed (°C/sec) | Workability 2T | Adhesion 2T | Corrosion resistance SST 1000 Hr | |
|---|---|---|---|---|---|
| | | | | flat part | 2T part |
| Present invention | 5 | 5 | 5 | 5 | 5 |
| | 10 | 5 | 5 | 5 | 5 |
| | 20 | 5 | 5 | 5 | 5 |
| | 30 | 5 | 5 | 5 | 5 |
| | 50 | 5 | 5 | 5 | 5 |
| The numerals of the evaluation results are the averages of the results. | | | | | |

### Example 15 (Preferred embodiments of the invention)

Prepainted steel sheets of the present invention were prepared and the properties of them were determined as follows to confirm the effect of the present invention.

Hot-dip zinc-aluminum alloy coated steel sheets were prepared in a hot dipping bath having the following composition (Example 1) and they were used as the materials:

The bath composition:

| | |
|---|---|
| Al concentration | 1.0 wt.% |
| Pb concentration | 0.005 wt.% |
| Si concentration | 0.01 wt.% |
| Zn concentration | the balance |

Then the sheets were subjected to chemical conversion treatment to form a coating film in various amounts on the materials (hot-dip zinc-aluminum alloy coated steel sheets with a chromate solution (type A) having a Cr to Si ratio of 55:45 which comprised a mixture of a solution containing silica having an average particle diameter of 10 m» (specific surface area: 200 m²/g) and a solution containing silica having an average particle diameter of 50 m» (specific surface area: 50 m²/g) in a ratio of 1:1; a chromate solution (type B) having a Cr to Si ratio of 55:45 comprising only the solution containing silica having an average particle diameter of 50 m» (specific surface area: 200 m²/g) or a phosphate solution.

Then an epoxy resin paint containing 15% of a rustproof pigment was applied to each of the treated zinc-aluminum alloy coated steel sheet. After baking at 210°C for 35 sec, an under-paint having a dry thickness of 3 » was given. Then an oil-free polyester resin paint as the top-painting paint was applied thereto and baked at 220°C for 45 sec to form a top-paint having a dry thickness of 11 ».

The scratch resistance, workability, adhesion and corrosion resistance of the prepared prepainted steel sheets were determined. The results are shown in Table 27 together with the conditions.

The scratch resistance was determined by applying a copper coin to the painted surface at an angle of 45° and moved under a load of 3 kg. The results were evaluated on the basis of the standard shown in Table 26.

The workability was determined by the 2T bend test in the same manner as that of Example 1 and the results were evaluated on the basis of the standard shown in Table 1.

The adhesion in the 2T part of the prepainted steel sheet was determined also in the same manner as that of Example 9 and the results were evaluated on the basis of the standard shown in Table 3.

The corrosion resistance test was conducted according to JIS Z 2371 in the same manner as that of Example 4. The flat part and 2T part of the prepainted steel sheet were subjected to the salt spray test (SST, 1000 Hr.). The results were evaluated on the basis of the standard shown in Table 6.

The prepainted steel sheets having not only excellent workability, adhesion and corrosion resistance but also an excellent scratch resistance could be prepared by the present invention.

**Table 26**

| (Standard of evaluation of scratch resistance) | |
|---|---|
| | Standard |
| 5 | The area of the exposed under-paint was less than 10% and no sheet was exposed. |
| 4 | The area of the exposed under-paint was 10 to 70% and no starting sheet was exposed. |
| 3 | The area of the exposed under-paint was more than 70% and that of the starting sheet was less than 30%. |
| 2 | The area of the exposed under-paint was 30 to 70%. |
| 1 | The area of the exposed under-paint was more than 70%. |

Those examples labelled "comparative" are less preferred.

The chromate solution of type A had a Cr to Si ratio of 55:45 and comprised a mixture of a solution containing silica having an average particle diameter of 10 m» (specific surface area: 200 m²/g) and that having an average particle diameter of 50 m» (specific surface area: 50 m²/g) in a ratio of 1:1.

The chromate solution of type B had a Cr to Si ratio of 55:45 and comprised only a solution containing silica having an average particle diameter of 50 m» (specific surface area: 200 m²/g).

The numerals of the evaluation results in the above Table are the averages of the results.

## Claims

1. A process for the preparation of a hot-dip zinc-aluminium alloy coated steel sheet suitable for a prepainted steel sheet, the process comprising coating a steel sheet in a hot dipping bath comprising 0.3 to 3.5 wt.% of Al, 100ppm or less of Pb and the balance of Zn and unavoidable impurities, wherein the temperature of the steel sheet dipped in the hot dipping bath is lower than that of the hot dipping bath by 10 to 80°C, taking the steel sheet out of the hot dipping bath and reheating the coated steel sheet to a temperature above the melting temperature of the coating layer.

2. A process according to Claim 1 wherein the hot dipping bath contains 1/100 to 1 part, per part of Al, of Si.

3. A process according to Claim 1 or 2 wherein the hot dipping bath contains 0.01 to 1.5 wt.% of Mg, Mn or Cu.

4. A process according to any preceding claim wherein the coated steel sheet is reheated to a temperature of from 420°C to 560°C.

5. A process according to any preceding claim additionally comprising cooling the hot-dip zinc-aluminium alloy coated steel sheet to the solidifying point thereof at a rate of at least 10°C/sec.

6. A process for the preparation of a prepainted steel sheet having an excellent workability and corrosion resistance comprising forming a layer by chemical conversion treatment and further a surface painting film layer on the hot-dip zinc-aluminium alloy coated steel sheet as prepared in any of Claims 1 to 5.

7. A hot-dip zinc-aluminium alloy coated steel sheet as prepared in any of Claims 1 to 5 and/or a prepainted steel sheet as prepared in Claim 6.

## Patentansprüche

1. Verfahren für die Herstellung eines durch Heiß-Tauchen mit einer Zinkaluminiumlegierung beschichteten Stahlblechs, geeignet für ein vorgestrichenes Stahlblech, wobei der Prozeß das Beschichten eines Stahlbleches in einem Heiß-Tauchbad mit 0,3 bis 3,5 Gew.% Aluminium, 100 ppm oder weniger Pb und den Ausgleich an Zn und unvermeidbaren Verunreinigungen umfaßt, wobei die Temperatur des Stahlbleches, das in das heiße Tauchbad getaucht wird, »m 10 bis 80 °C niedriger ist als diejenige des Tauchbades, Herausnehmen des Stahlbleches aus dem Tauchbad und Wideraufheizen des beschichteten Stahlbleches auf eine Temperatur oberhalb der Schmelztemperatur der Beschichtungsschicht.

2. Verfahren nach Anspruch 1, wobei das Tauchbad pro Teil Al 1/100 zu 1 Teil Si enthält.

3. Verfahren nach Anpruch 1 oder 2, wobei das Tauchbad 0,01 bis 1,5 Gew.% Mg, Mn oder Cu enthält.

4. Verfahren nach einem der vorhergehenden Ansprüche, wobei das beschichtete Stahlblech auf eine Temperatur von 420 °C bis 560 °C wieder aufgeheizt wird.

5. Verfahren nach einem der vorhergehenden Ansprüche, der zusätzlich ein Abkühlen des durch Tauchüberzug mit Zinkaluminium beschichteten Stahlbleches auf dessen Härtetemperatur mit einer Geschwindigkeit von zumindest 10 °C/sek umfaßt.

6. Verfahren für die Herstellung eines vorgestrichenen Stahlbleches mit einer exzellenten Bearbeitbarkeit und Korosionswiderstand, das die Ausbildung einer Schicht durch chemische Unwandlungsbehandlung umfaßt sowie weiterhin eine Oberflächenstreichfilmschicht auf dem durch Tauchüberzug mit einer Zinkaluminiumlegierung beschichteten Stahlblech, wie in einem der Ansprüche 1 bis 5 hergestellt.

7. Durch Tauchüberzug mit einer zinkaluminiumlegierung beschichtetes Stahlblech wie in einem der Ansprüche 1 bis 5 hergestellt und/oder ein vorgestrichenes Stahlblech, wie in Anspruch 6 hergestellt.

## Revendications

1. Procédé pour la préparation d'une tôle d'acier revêtue d'un alliage de zinc-aluminium par immersion à chaud, convenant pour une tôle d'acier prépeinte, le procédé consistant à revêtir une tôle d'acier dans un bain d'immersion chaud comprenant 0,3 à 3,5% en poids de Al, 100 ppm ou moins de Pb et pour le reste, du Zn et des impuretés inévitables, dans lequel la température de la tôle d'acier immergée dans le bain d'immersion chaud est inférieure à celle du bain d'immersion chaud de 10 à 80°C, à retirer la tôle d'acier du bain d'immersion chaud et à réchauffer la tôle d'acier revêtue à une température supérieure à la température de fusion de la couche de revêtement.

2. Procédé suivant la revendication 1, dans lequel le bain d'immersion chaud contient 0,01 à 1 partie de Si par partie de Al.

3. Procédé suivant la revendication 1 ou 2, dans lequel le bain d'immersion chaud contient 0,01 à 1,5% en poids de Mg, Mn ou Cu.

4. Procédé suivant l'une quelconque des revendications précédentes, dans lequel la tôle d'acier revêtue est réchauffée à une température allant de 420°C à 560°C.

5. Procédé suivant l'une quelconque des revendications précédentes, consistant de plus à refroidir la tôle d'acier, revêtue d'un alliage de zinc-aluminium par immersion à chaud, jusqu'à son point de solidification à une vitesse d'au moins 10°C par seconde.

6. Procédé pour la préparation d'une tôle d'acier prépeinte présentant une aptitude au façonnage et une résistance à la corrosion excellentes, consistant à former une couche par traitement de transformation chimique et, en outre, une couche de pellicule de peinture de surface sur la tôle d'acier, revêtue d'un alliage de zinc-aluminium par immersion à chaud, telle que préparée suivant l'une quelconque des revendications 1 à 5.

7. Tôle d'acier revêtue d'un alliage de zinc-aluminium par immersion à chaud, telle que préparée suivant l'une quelconque des revendications 1 à 5 et/ou tôle d'acier prépeinte telle que préparée suivant la revendication 6.
